# EUROPEAN PATENT SPECIFICATION

(11) **EP 3 351 610 B1**
(45) Date of publication and mention of the grant of the patent: **07.10.2020**
(21) Application number: 16846753.8
(22) Date of filing: 11.08.2016
(51) Int. Cl.: C10L 1/10, C10L 1/08, C10L 10/02, C10L 1/12, C10L 1/14

(54) **FUEL ADDITIVE FOR REDUCING GREENHOUSE GASES, NITROGEN OXIDES AND PARTICULATE MATTER**
TREIBSTOFFADDITIV ZUR VERRINGERUNG VON TREIBHAUSGASEN, STICKOXIDEN UND FEINSTAUB
ADDITIF POUR COMBUSTIBLE DESTINÉ À RÉDUIRE LES GAZ À EFFET DE SERRE, LES OXYDES D'AZOTE ET LA MATIÈRE PARTICULAIRE

(30) Priority: 17.09.2015 KR 20150131375
(43) Date of publication of application: 25.07.2018
(73) Proprietor: Lee, Young Seo, Paju-si, Gyeonggi-do 10854 (KR); Lee, Myeong Jin, Gunpo-si, Gyeonggi-do 15863 (KR)
(72) Inventor: Lee, Young Seo, Paju-si, Gyeonggi-do 10854 (KR); Lee, Myeong Jin, Gunpo-si, Gyeonggi-do 15863 (KR)
(74) Representative: Ter Meer Steinmeister & Partner
(86) International application number: PCT/KR2016/008816
(87) International publication number: WO 2017/047932

(56) References cited:
- EP-A2- 0 212 922
- WO-A1-98/26028
- CA-A1- 2 208 279
- KR-A- 20090 105 925
- KR-B1- 100 569 899
- KR-B1- 101 071 204
- US-A- 4 839 094
- US-A- 5 766 272
- US-A1- 2014 000 156

## Description

### [Technical Field]

The present disclosure relates to a fuel additive capable of reducing the generation of greenhouse gases, nitrogen oxides, and particulate matter and improving combustion efficiency by being added to a heavy fuel oil during combustion in an internal combustion engine or a boiler using a heavy fuel oil as fuel.

### [Background Art]

In order to slow down global warming, IMO MEPC has proposed to lower ship speed and sail as a way of reducing CO2 which is the GHG (Green House Gas) emitted by ships. In order to reduce fuel costs, shipping companies also voluntarily lower steaming, and most of the container ships engaged in international voyages are lowering streaming. In addition, the increase in the shipping volume, which is increasing day by day, increases the burden on the fuel cost of the ship, and thus the development of fuel cost reduction technology is urgently required.

Most ships using two stroke large diesel engines operating on international voyages use a heavy fuel oil for ships. Since the heavy fuel oil has a high kinematic viscosity, there is a disadvantage in that it cannot be used unless heated to 100°C or higher. In order to lower the kinematic viscosity of heavy fuel oil with a high kinematic viscosity, which is a disadvantage, Ryu et al. made an attempt to study to lower the kinematic viscosity of heavy fuel oil by mixing it with dimethyl ether having a low kinematic viscosity. As a result, the kinematic viscosity of heavy fuel oil was lowered and applied to a diesel engine for ships without heating. In this study, it was confirmed that engine performance can also be improved by using a heavy fuel oil mixed with dimethyl ether which is attracting attention as an alternative fuel for a diesel engine. In addition, many studies and demonstrations have been made on fuel additives for diesel engines in various fields.

Fuel cost accounts for a large part of the budget expenditure of shipping companies operating and managing ships. Most domestic and overseas shipping companies are sailing ships by lowering ship speed to save fuel costs. However, when low-load operation continues for a long time in a state where a high-output engine is mounted, there arises a problem that maintenance costs are increased due to generation of carbon and increase in failure rate due to incomplete combustion. In addition, the burden on the fuel cost of ships increasing day by day urgently requires the development of technology to save fuel cost to shipowners.

In order to solve these problems, researches on fuel additives that can minimize the generation of residual carbon powder, dust, or sulfur dust, etc. in the combustion of heavy fuel oil or improve the combustion efficiency have been made intermittently. For example, Korean Patent Registration Publication No. 10-0743826 discloses a fuel additive for a bituminous heavy fuel oil/water emulsion including 30 to 60% by weight of magnesium hydroxide having a particle size of 0.1 to 10 µm; 0.1 to 1% by weight of polycarboxylic acid and/or its salt; and the water of the remaining % by weight.

In addition, Korean Patent Registration Publication No. 10-1071204 discloses a fuel additive for a heavy fuel oil consisting of a composition including 25 to 55% by weight of an oil soluble metallic compound including any one of calcium, barium, manganese or iron, 15 to 25% by weight of alcohol, 10 to 20% by weight of hydrotreated light distillate, 5 to 15% by weight of kerosene, 5 to 15% by weight of mineral oil, and 2 to 8% by weight of non-ionic surfactant, in which the mineral oil is composed of one or more kinds selected from the group consisting of a hydrotreated heavy paraffinic distillate or a hydrotreated light paraffinic distillate, solvent-dewaxed heavy paraffinic distillate, solvent-dewaxed light paraffinic distillate, hydrotreated and dewaxed heavy paraffinic distillate, and hydrotreated and dewaxed light paraffinic distillate. US2014/000156 relates to a fuel additive for heavy oil.

### [Disclosure]

### [Technical Problem]

The present disclosure has been made under the background of the prior art, and an object of the present disclosure is to provide a method for reducing the generation of greenhouse gases, nitrogen oxides and particulate matter added to a heavy fuel oil during combustion in an internal combustion engine or a boiler using a heavy fuel oil as fuel, and to provide a fuel additive capable of improving combustion efficiency.

### [Technical Solution]

In order to achieve the above object, one aspect of the present disclosure provides a fuel additive for a heavy fuel oil in the form of a composition including an oil soluble metallic compound, an oxygen supplier, a dispersant, a lubricant, a non-ionic surfactant, and a detergent. Hereinafter, the fuel additive for a heavy fuel oil according to the present disclosure will be described separately for each constituent component.

### Oil soluble metallic compound

The oil soluble metallic compound, which is one of the components of the fuel additive for a heavy fuel oil according to the present disclosure, increases the reactivity with oxygen during the combustion of heavy fuel oil, which is fuel oil, accelerates the oxidation and promotes the combustion reaction of low combustibility components such as asphaltenes, and acts as a combustion promoter for suppressing generation of exhaust gas and dust. In the present disclosure, the oil soluble metallic compound preferably includes a metal having a high combustion promoting reactivity, and at the same time has a property of being oil soluble in fuel-derived heavy oil. Examples of the metal having a high combustion promoting reactivity include calcium, barium, manganese or iron, etc. In the present disclosure, it is preferable that the oil soluble metallic compound is composed of an active metal portion and an organic ligand in order to be well dissolved in fuel-derived heavy oil. Examples of the oil soluble metallic compound include calcium acetylacetonate, calcium naphthenate, calcium oxlate, barium acetylacetonate, barium naphthenate, barium oxlate, manganese acetylacetonate, manganese naphthenate, manganese oxlate, iron acetylacetonate, iron naphthenate, iron oxlate, etc. In addition, in the present disclosure, the oil soluble metallic compound may be a metal salt of a carboxylic acid or a metal salt of a sulfonic acid from a different viewpoint.

In consideration of the relative size of the combustion promoting reactivity, the oil soluble metallic compound in the present disclosure is an oil soluble metallic compound including calcium. The calcium salt of the sulfonic acid is a calcium alkylbenzenesulfonate including a double alkylaryl group. The alkyl group of the calcium alkylbenzenesulfonate is characterized by having 8 to 50 carbon atoms. A specific example of the calcium alkylbenzenesulfonate is calcium dodecylbenzenesulfonate, which is a typical anionic surfactant.

In the fuel additive for a heavy fuel oil according to the present disclosure, the content of the oil soluble metallic compound is 20 to 25 wt% based on the total weight of the composition, considering the effect of minimizing dust generation and compatibility with other constituents.

### Oxygen carrier

Even if excessive combustion air is supplied during heavy fuel oil combustion, the rate of exhaustion by the combustion reaction such as heterogeneous surface reaction is higher than the diffusion rate of oxygen, so that the oxygen concentration becomes thin at the interface where the combustion reaction occurs, thereby causing an oxygen deficiency phenomenon. The oxygen carrier which is one component of the fuel additive for a heavy fuel oil according to the present disclosure is preferably a compound having a low boiling point. The low boiling point compound can contribute to complete combustion by increasing the combustion reaction surface area by the vaporization phenomenon inside a burner spray droplet.

The low boiling point compound used as an oxygen carrier in the present disclosure is dimethyl carbonate, diethyl carbonate, diisopropyl carbonate, diisopropyl carbonate, dibutyl carbonate, dipentyl carbonate, methylethyl carbonate, methylpropyl carbonate, or ethypropyl carbonate.

In the fuel additive for a heavy fuel oil according to the present disclosure, the content of the oxygen carrier is 30 to 35% by weight based on the total weight of the composition, considering the effect of minimizing dust generation and compatibility with other components.

### Dispersant

The dispersant, which is one component of the fuel additive for a heavy fuel oil according to the present disclosure, plays as a role in preventing the formation of sludge, lowering the flash point of the heavy fuel oil, and reducing the kinematic viscosity and surface tension. When the viscosity and the surface tension of the heavy fuel oil are reduced, the particle diameter of the fuel becomes atomized and homogenized at the time of injection from the nozzle, and it is possible to lower the temperature of the exhaust gas of the internal combustion engine by the rapid combustion and the low temperature explosion at the time of combustion. In the present disclosure, the dispersant is a hydrotreated light distillate.

Hydrotreated is a treatment method of adding hydrogen to oil, etc. In addition, the light distillate refers to a light hydrocarbon which is distilled first when the crude oil is distilled. The hydrotreated light distillate has a boiling point of usually 150 to 300°C, but is not limited thereto. The hydrotreated light distillate which can be used in the present disclosure includes products such as CAS Registration Nos. 64742-47-8 and 68921-07-3, but is not limited thereto.

In the fuel additive for a heavy fuel oil according to the present disclosure, the content of the hydrotreated light distillate is 15 to 20% by weight based on the total weight of the composition, considering the effect of reducing the flash point and the kinematic viscosity, minimizing the generation of dust and residual carbon powder and the compatibility with other components.

### Lubricant

The lubricant, which is one component of the fuel additive for a heavy fuel oil according to the present disclosure, plays a role in maintaining the shape of sludge redispersed in the form of microparticles and suppressing the occurrence of friction in an internal combustion engine. In the present disclosure, the lubricant is preferably a paraffinic oil, more preferably modified by hydrotreating or dewaxing treatment. The paraffinic oil modified by the hydrotreating or dewaxing treatment may be composed of at least one selected from the group consisting of a hydrotreated heavy paraffinic distillate (CAS Registration No. 64742-54-7), a hydrotreated light paraffinic distillate (CAS Registration No. 64742-55-8), a solvent-dewaxed heavy paraffinic distillate (CAS Registration No. 64742-65-0), a solvent-dewaxed light paraffinic distillate (CAS Registration No. 64742-56-9), a hydrotreated and dewaxed heavy paraffinic distillate (CAS Registration No. 91995-39-0) or a hydrotreated and dewaxed light paraffinic distillate (CAS Registration No. 91995-40-3), but is not limited thereto.

In the fuel additive for a heavy fuel oil according to the present disclosure, the content of the lubricant is 3 to 7% by weight based on the total weight of the composition, considering the effect of reducing the flash point and the kinematic viscosity, minimizing the generation of dust and residual carbon powder and the compatibility with other components.

### Non-ionic surfactant

The non-ionic surfactant, which is one component of the fuel additive for a heavy fuel oil according to the present disclosure, plays a role in preventing the formation of sludge and redispersing the generated sludge into a microparticle. In particular, the non-ionic surfactant exhibits a repulsion due to steric hindrance to form a stable dispersion system. When used in combination with an ionic material such as an oil soluble metallic compound, dispersion performance is greatly improved.

The non-ionic surfactant used in the present disclosure is not greatly limited in its kinds such as ester base, ether base, fatty acid amide base, aliphatic amine derivative, and the like. Examples of the ester-based non-ionic surfactant include sorbitan esters of fatty acids, pentaerythritol esters of fatty acids, propyleneglycol monoesters of fatty acids, glycerin monoesters of fatty acids, polyethyleneglycol sorbitan esters of fatty acids, polyethyleneglycol sorbitol esters of fatty acids, and polyethyleneglycol esters of fatty acids, and the like. Examples of the ether-based non-ionic surfactant include polyoxyethylene alkyl ethers, polyoxyethylene alkyl phenyl ethers, alkylpolyglycosides, and the like. Examples of the fatty acid amide-based non-ionic surfactant include fatty acid dialkanolamides, fatty acid monoalkanolamides, polyoxyethylene fatty acid amides, and the like. Examples of the aliphatic amine derivative non-ionic surfactant include polyoxyethylene alkylamine, and the like. Considering the effect of reducing the flash point and the kinematic viscosity, minimizing the generation of dust and residual carbon powder and the compatibility with other components, the non-ionic surfactant used in the present disclosure is composed of at least one selected from the group consisting of sorbitan esters of fatty acids, polyethyleneglycol esters of fatty acids, or polyethylene glycol sorbitan esters of fatty acids.

Examples of sorbitan esters of fatty acids include sorbitan monooleate, sorbitan monolaurate, and the like. Examples of the polyethyleneglycol sorbitan esters of fatty acids include polyethylene glycol sorbitan monooleate, and the like. Examples of the polyethyleneglycol esters of fatty acids include polyethylene glycol dilaurate, polyethylene glycol monooleate, polyethylene glycol dioleate, polyethylene glycol monoricinoleate, polyethylene glycol monostearate, and the like.

In the fuel additive for a heavy fuel oil according to the present disclosure, the content of the non-ionic surfactant is preferably 8 to 15% by weight based on the total weight of the composition, considering the effect of reducing the flash point and the kinematic viscosity, minimizing the generation of dust and residual carbon powder and the compatibility with other components.

### Detergent

The detergent, which is one component of the fuel additive for a heavy fuel oil according to the present disclosure, plays a role in decomposing the secondary oxide and the combustion products to reduce the formation of precipitates on the surface of the metal parts surface. The detergent may be composed of at least one selected from the group consisting of alkaline metal salts of a known sulfonate, alkaline earth metal salts of sulfonates, alkaline metal salts of phenates, alkaline earth metal salts of phenates, alkaline metal salts of salicylates, alkaline earth metal salts of salicylates, alkaline metal salts of naphthenate, or alkaline earth metal salts of naphthenate. The alkaline metal or alkaline earth metal is preferably selected from calcium, magnesium, sodium, or barium.

The metal salt-type detergent may include a metal in a stoichiometric amount or in excess thereof. In the latter case, it is treated as an overbased detergent. The overbased detergent is a metal salt that dissolves in oil and appears as a micelle consisting of an insoluble metal salt trapped in a suspension in a fuel oil composition described later. The overbased characteristic of the detergent is characterized by total base number (TBN), measured in accordance with ASTM D2896 standard, and is expressed in mg of KOH per gram. The overbased detergent itself typically has a TBN value of about 150 or more, or 250 or 450 or more. In the present disclosure, it is preferable that the detergent is an overbased detergent in consideration of the synergistic effect with other components. In addition, in the present disclosure, the TBN of the overbased detergent is preferably 200 or more, more preferably 300 or more. The overbasing process is well known in the pertinent art and typically involves reacting an acidic material with a reaction mixture including an organic acid or metal salt thereof, or a metal compound. The acidic material may be a gas such as carbon dioxide or sulfur dioxide, or it may be boric acid. A method for preparing an overbased alkaline metal sulfonate and phenate is described in U.S. Patent No. 4,839,094. A suitable method for an overbased sodium sulfonate is described in EP-A-235929. A method for preparing an overbased salicylate is described in U.S. Patent No. 5,451,331. In addition, commercially available overbased detergents include T106 (Overbased Heavy alkyl benzene synthetic calcium sulfonate of Anneng Chemical Co., Ltd. (CAS registration no. 61789-86-4)), CALCINATE™ C-300CS of Chemtura Corporation, OLOA 246S (Sulfonic acids, petroleum, calcium salts, overbased (CAS Registration No. 68783-96-0)) of Chevron Chemical Company, and the like. In addition, the overbased sulfonate-based detergent of CAS Registration No. 68783-96-0 has the structure of the following Formula 1, and the overbased sulfonate-based detergent of CAS Registration No. 115733-10-3 has the structure of the following Formula 2.

In the fuel additive for a heavy fuel oil according to the present disclosure, the content thereof is 7 to 15% by weight based on the total weight of the composition, considering the effect of improving combustion of the detergent, reducing NOx, minimizing the generation of dust and residual carbon powder and the compatibility with other components.

In addition, another aspect of the present disclosure relates to a fuel oil based on a heavy fuel oil, in which the fuel oil based on a heavy fuel oil according to the present disclosure includes a heavy fuel oil and the above-described fuel additives for a heavy fuel oil. At this time, the heavy fuel oil is not limited in its kind, and may be a heavy oil A, a heavy oil B, a heavy oil C (or bunker C oil), or a mixed heavy oil thereof. In addition, the content of the fuel additive for a heavy fuel oil in the fuel oil is not limited to a great extent. However, considering the effect of reducing the flash point and the kinematic viscosity of fuel additives, minimizing the generation of dust and residual carbon powder, reducing NOx and improving combustion efficiency, and the economic feasibility of a fuel oil, it is preferably 0.001 to 0.5 parts by weight, more preferably 0.005 to 0.1 parts by weight, per 100 parts by weight of the heavy fuel oil.

### [Advantageous Effects]

If a small amount (0.025%) of the fuel additive of the present disclosure is added to a heavy fuel oil, the generation of particulate matter (PM), residual carbons, nitrogen oxides and the like upon combustion can be reduced. In addition, if a small amount (0.025%) of the fuel additives of the present disclosure is added to a heavy fuel oil, the combustion efficiency can be enhanced since upon combustion, a maximum combustion pressure is increased, whereas an exhaust temperature is lowered. Thus, the fuel additive of the present disclosure is very useful for a large boiler using a heavy fuel oil as fuel, in particular, a large diesel engine.

### [Description of Drawings]

FIG. 1 is a schematic diagram of an experimental apparatus for an engine used in this study.
FIG. 2 is a graph illustrating the increase and decrease ratio of the output at each load depending on whether the fuel additive is added in the present study.
FIG. 3 is a graph illustrating the results of the fuel consumption rate depending on whether the fuel additive is added in the present study.
FIG. 4 is a graph illustrating the results of the maximum combustion pressure of the engine depending on whether the fuel additive is added in the present study.
FIG. 5 is a graph illustrating the exhaust temperatures after combustion of the engine at various loads depending on whether the fuel additive is added in the present study.

### [Detailed Description of Embodiment]

Hereinafter, the present disclosure will be described in more detail with reference to examples. However, the following examples are intended to clearly illustrate the technical features of the present disclosure and do not limit the scope of protection of the present disclosure.

The applicant of the present disclosure attempted to reduce the fuel cost by injecting a predetermined fuel additive (including an oil-soluble calcium-based organometallic compound as one component) into a heavy fuel oil for ships. Specifically, a method of reducing a fuel cost by injecting a predetermined amount of a fuel additive (including an oil-soluble calcium-based organometallic compound as one component) (0.025% of a fuel amount used) was tried. For the accuracy of the experiment, a two-stroke large diesel engine installed in the land-based power plant was an experiment object. The experimental engine load was divided into low, medium and high load (50, 75, 100%). The engine performance (output, fuel consumption rate, maximum combustion pressure (P-max), exhaust temperature) before and after the injection of fuel additives was compared and analyzed. Through this experiment, it was confirmed that the addition of the fuel additive reduced the fuel cost by 2% or more at the low load (50%), and that the maximum combustion pressure was increased while the exhaust temperature was lowered. Hereinafter, the research conducted by the applicant of the present disclosure will be described in detail.

### 1. Preparation of fuel additives used in experiments

23 parts by weight of calcium alkylbenzenesulfonate (Benzenesulfonic acid, mono-C15-30-branched alkyl and di-C11-13-branched and linear alkyl derivs., calcium salts; CAS Registration No. 71486-79-8), 32 parts by weight of dimethyl carbonate, 18 parts by weight of a hydrotreated light distillate (CAS Registration No. 64742-47-8), 5 parts by weight of a hydrotreated heavy paraffinic distillate (CAS Registration No. 64742-54-7), 12 parts by weight of sorbitan monooleate (CAS Registration No. 1338-43-8) and 10 parts by weight of an overbased calcium sulfonate detergent (Benzenesulfonic acid, C14-24-branched and linear alkyl derivatives, calcium salts, overbased; CAS Registration No. 115733-10-3) were mixed and stirred to prepare a fuel additive including an oil-soluble calcium-based organometallic compound.

### 2. Experimental apparatus and method

In this study, for the accuracy of the experiment, a two-stroke large diesel engine installed in the land-based power plant was an experiment object. The fuel additives were injected at a rate of 0.025% of the fuel used to perform an experiment. The experiments were carried out after the load of the experimental engine had a stable thermal equilibrium at the exhaust temperature, and was divided into three stages: low, medium and high load (50, 75, 100%) for the experiments. It was maintained constant within the range of ±3% of Load Limiter, and the generator output voltage was maintained and driven at the rated voltage. And the engine performance (output, fuel consumption rate, maximum combustion pressure (P-max), exhaust temperature) before and after the injection of fuel additives was compared and analyzed. Table 1 exihibits the specifications of the experimental engine used in this study. The equipment to be applied for the performance experiment is Diesel Engine Generator equipment manufactured and installed by Doosan Engine Co., Ltd, and is a 40MW generator. And Table 2 exihibits the properties of the fuels used in this study and exihibits the fuel properties of heavy fuel oil after injecting fuel additives at 0.025% ratio of heavy fuel oil and the fuel properties of heavy fuel oil before injecting them into a heavy fuel oil for ships. As the fuel additive, an additive including an oil-soluble calcium-based organometallic compound was used. To analyze the fuel composition of each fuel, three samples were collected during the experiment to analyze the exact composition of the fuel. The analysis was commissioned by a domestic fuel analysis agency

**[Table 1]**

| Item | Description |
|---|---|
| Engine type | Low speed two stroke cycle, 12K80MC-S |
| Bore × Stroke | 800mm ×2300mm |
| Combustion type | Direct injection type |
| No. of cylinders | 12 |
| MCR output | 41,320 kW |
| MCR rpm | 109.1 rpm |
| Mean effective pressure | 16.4 kg_{f}/cm² |
| Mean piston speed | 8.36 m/s |
| Weight | 1,413 ton |
| Turbo charger rpm | 11,000 rpm |
| Firing order | 1-5-12-7-2-6-10-3-8-4-11-9 |

**[Table 2]**

| Item | Heavy fuel oil | Added fuel oil |
|---|---|---|
| Density at 15°C, g/mℓ | 0.9384 | 0.9378 |
| Ash, mass% | 0.042 | 0.030 |
| Sulfur, mass% | 0.254 | 0.273 |
| Viscosity at 100°C, mm²/s | 24.27 | 23.39 |
| Water by distillation, volume% | 0.10 | 0.20 |
| Nitrogen, mass% | 0.33 | 0.32 |
| Gross calorific value, kcal/kg | 10,550 | 10,546 |
| Net calorific value, kcal/kg | 9,940 | 9,934 |
| Carbon, mass% | 86.68 | 86.56 |
| Hydrogen, mass% | 12.04 | 12.07 |
| Oxygen, mass% | 0.65 | 0.75 |

| | | |
|---|---|---|
| * Heavy fuel oil: Heavy fuel oil before injecting fuel additives * Added fuel oil: Heavy fuel oil into which fuel additives are injected at a ratio of 0.025% | | |

The fuel additive injection system installed a dosing pump that can automatically supply a certain amount around the control tank, and the supply position is connected to a supply piping so that it can be supplied to the top of the fuel control tank. In addition, the engine output was measured in a local integrated watt-hour meter and a control room meter, and the fuel consumption amount was referred to an on-site mass flowmeter reading installed on the fuel oil supply line side. Table 3 exihibits the dosing pump and mass flowmeter specifications. In calculating the engine output and fuel consumption rate, each item on the performance was calculated by applying the calibration curve and formula given by the manufacturer. FIG. 1 is a schematic diagram of an experimental apparatus for an engine used in this study.

**[Table 3]**

| Item | Description |
|---|---|
| Dosing pump | CMG Techwin, AX1-12 model, 110 ml/min |
| Mass flowmeter | Endress Hauser, IP67/NEMA/TYPE4X model |

### 3. Experimental results and consideration

### 3.1 Engine power output

The engine output was measured by dividing them into three stages of low, medium and high load (50, 75, 100%). At the low load of 50% of the engine load, the average value measured 4 times is exihibited. At the medium load of 75% and the high load of 100% of the engine load, the average value measured 7 times is exihibited. Table 4 exihibitsthe rate of increase and decrease of the output at each load, and FIG. 2 illustrates the results thereof in the form of a graph. At a low load of 50%, the output decreased by about 2.1%, but increased by about 1.6% and 0.4% at 75% of medium load and 100% of high load, respectively. These results indicate that the output is improved by completely combusting the unburned matter with the fuel additive effect at a load of 75% or more. This engine output value is a value obtained by calibrating the measured output value with the design Gen power factor value. These results exihibitthat the engine power is improved in medium and heavy load regions rather than in a low load when the fuel additive is injected into a heavy fuel oil.

**[Table 4]**

| Load(%) | HFO(kW) | Added fuel(kW) | Difference | Ratio(%) |
|---|---|---|---|---|
| 50 | 21,186 | 20,748 | -438 | -2.11 |
| 75 | 30,521 | 31,016 | 495 | 1.60 |
| 100 | 40,460 | 40,605 | 145 | 0.36 |

| | | | | |
|---|---|---|---|---|
| * HFO: Heavy fuel oil before injecting fuel additives * Added fuel: Heavy fuel oil into which fuel additives are injected at a ratio of 0.025% | | | | |

### 3.2 Fuel consumption rate

Table 5 and FIG. 3 exhibit the results of the fuel consumption rate. At the low load of 50% of the engine load, the average value measured 4 times is exihibited. At the medium load of 75% and the high load of 100% of the engine load, the average value measured 7 times is exihibited. At a low load, the fuel consumption rate decreased by about 2.2%, and decreased by about 0.7% and 0.8% of medium and high loads. It is determined that these results are produced by combustion promotion. That is, it was confirmed that the fuel efficiency was improved at full load by injecting the fuel additive into the heavy fuel oil. In particular, the fuel consumption reduction rate was higher at low load than at medium and high load regions.

**[Table 5]**

| Load(%) | HFO(g/kWh) | Added fuel(g/kWh) | Difference | Ratio(%) |
|---|---|---|---|---|
| 50 | 207.430 | 202.833 | -4.597 | -2.27 |
| 75 | 186.395 | 185.103 | -1.292 | -0.70 |
| 100 | 188.422 | 186.913 | -1.509 | -0.81 |

| | | | | |
|---|---|---|---|---|
| * HFO: Heavy fuel oil before injecting fuel additives * Added fuel: Heavy fuel oil into which fuel additives are injected at a ratio of 0.025% | | | | |

### 3.3 Maximum combustion pressure (P-max)

Table 6 and FIG. 4 exhibit the results of the maximum combustion pressure of the engine. Each value was measured after all cylinders 12 cylinders were measured, and the average value was exihibited. The maximum combustion pressure increased about 3.0% at low load and increased about 6.6% and 0.9% at medium and high load, respectively. That is, it was confirmed that the maximum combustion pressure was increased at full load by injecting the fuel additive into the heavy fuel oil for ships. In particular, it exhibits a large increase rate in medium load of 75%, which is the commercial load of the engine. As exihibitedin Table 2, it is analyzed that engine combustion is promoted actively by the action of oxygen included in the fuel additive, thereby improving combustion.

**[Table 6]**

| Load(%) | HFO(Bar) | Added fuel(Bar) | Difference | Ratio(%) |
|---|---|---|---|---|
| 50 | 86.25 | 88.83 | 2.58 | 2.90 |
| 75 | 114.83 | 122.91 | 8.08 | 6.57 |
| 100 | 139.83 | 141.08 | 1.25 | 0.89 |

| | | | | |
|---|---|---|---|---|
| * HFO: Heavy fuel oil before injecting fuel additives * Added fuel: Heavy fuel oil into which fuel additives are injected at a ratio of 0.025% | | | | |

### 3.4. Exhaust temperature

Table 7 and FIG. 5 exhibit the post-combustion temperature of the engine at each load. Each value was measured after all cylinders 12 cylinders were measured, and the average value was exhibited. At the low load, the exhaust temperature decreased by about 2.7%, and at medium and high loads, it decreased by about 2.4% and 0.6%. That is, it was confirmed that the exhaust temperature decreases at full load by injecting the fuel additive into the heavy fuel oil. It is determined that the asphalt and sludge included in the heavy fuel oil are well dispersed by the dispersant included in the fuel additive, thereby producing the fuel atomization and homogenization effect of fuel during the fuel injection so as to be stable combustion.

**[Table 7]**

| Load(%) | HFO(°C) | Added fuel(°C) | Difference | Ratio(%) |
|---|---|---|---|---|
| 50 | 337.08 | 328.08 | -9.00 | -2.74 |
| 75 | 326.42 | 318.83 | -7.59 | -2.38 |
| 100 | 343.08 | 341.17 | -1.91 | -0.56 |

| | | | | |
|---|---|---|---|---|
| * HFO: Heavy fuel oil before injecting fuel additives * Added fuel: Heavy fuel oil into which fuel additives are injected at a ratio of 0.025% | | | | |

### 4. Conclusion

In this study, a two-stroke high-power large diesel engine was tested using a standardized measurement equipment on the land that is not affected by the ocean and weather conditions. In order to compare and analyze the engine performance (engine output, fuel consumption rate, maximum combustion pressure, exhaust temperature) before and after injection into the fuel additive of heavy fuel oil for ships, experiments were carried out at low, medium and high loads (50, 75, 100%) of the engine, and the following research results were obtained.
(1) At low loads with 50% engine load, the output decreased by about 2.1%, but increased by about 1.6% and 0.4% at 75% medium load and 100% high load of an engine load, respectively. These results exhibit that the engine output is improved in medium and heavy load regions rather than in low load when the fuel additive is injected into a heavy fuel oil.
(2) Fuel consumption rate decreased by about 2.2% at low load and about 0.7% and 0.8% at medium and high load, respectively. That is, it was confirmed that the fuel efficiency was improved at full load by injecting the fuel additive into the heavy fuel oil. In particular, the fuel consumption reduction rate was higher at low load than at medium and high load regions.
(3) The maximum combustion pressure increased by about 3.0% at low load, and about 6.6% and 0.9% at medium and high loads, respectively. That is, it was confirmed that the maximum combustion pressure was increased at full load by injecting the fuel additive into the heavy fuel oil for ships.
(4) As a result of measurement of exhaust temperature, it decreased by about 2.7% at low load, about 2.4% at medium load, and about 0.6% at high load. That is, it was confirmed that the exhaust temperature decreases at full load by injecting the fuel additive into the heavy fuel oil. It is determined that the fuel additive influences the engine combustion, so that it becomes stable combustion.

Through this study, it was confirmed that the fuel cost can be reduced by 2% or more at the low load (50%) by injecting the predetermined fuel additive including the oil soluble calcium-based organometallic compound into a heavy fuel oil for ships which is currently used in the two-stroke high-power large diesel engine. In can be understood that the maximum combustion pressure increases, whereas the exhaust temperature is lowered. Through these results, it is thought that the engine performance is improved. Accordingly, it is possible to reduce fuel costs by injecting a fuel additive into a two-stroke large diesel engine which uses a heavy fuel oil for ships.

### 5. Additional experiments

In addition to the above studies, the changes in exhaust emissions due to the addition of fuel additives were observed, and the results are exhibited in Tables 8 and 9 below. Table 8 exhibits the emission changes of nitrogen oxide (NOx) according to the addition of the fuel additive and Table 9 exhibits the emission change of particulate matter (PM) according to the addition of the fuel additive. As exhibited in Tables 8 and 9, when the fuel additive of the present disclosure is added to a heavy fuel oil and burned, the generation of nitrogen oxides and particulate matter is greatly reduced.

**[Table 8]**

| load - | NOx emission amount before injecting a fuel additive (g/kWh) | NOx emission amount after injecting a fuel additive (g/kWh) | Reduction rate of NOx emission amount according to the injection of a fuel additive (%) |
|---|---|---|---|
| 50% | 16.6 | 12.6 | -24 |
| 7 5 % | 21.5 | 11.7 | -46 |
| 100% | 22.4 | 14.3 | -36 |
| Average reduction rate of NOx emission amount according to the injection of a fuel additive(%) | | | -35 |

**[Table 9]**

| load | PM emission amount before injecting a fuel additive(mg/m³) | PM emission amount after injecting a fuel additive(mg/m³) | Reduction rate of PM emission_amount_ according to the injection of a fuel additive (%) |
|---|---|---|---|
| 50% | 64.1 | 27.3 | -57.4 |
| 75% | 100.8 | 40.9 | -59.4 |
| 100% | 108.6 | 43.8 | -59.7 |
| Average reduction rate of PM emission amount according to the injection of a fuel additive (%) | | | -58.8 |

From the foregoing, the present disclosure has been described by way of the above examples, but is not limited thereto. Therefore, the protection scope of the present disclosure should be construed as including all embodiments falling within the scope of the appended claims.

## Claims

1. A fuel additive for a heavy fuel oil in composition form, the fuel additive comprising:
20 to 25% by weight of an oil soluble metallic compound; 30 to 35% by weight of an oxygen carrier; 15 to 20% by weight of a dispersant; 3 to 7% by weight of a lubricant; 8 to 15% by weight of a non-ionic surfactant; and 7 to 15% by weight of an overbased sulfonate-based a detergent, based on the total weight of the composition,
wherein the oil soluble metallic compound is a calcium alkylbenzenesulfonate and the alkyl group has 8 to 50 carbon atoms,
wherein the oxygen carrier is composed of at least one selected from the group consisting of dimethyl carbonate, diethyl carbonate, dipropyl carbonate, diiosopropyl carbonate, dibutyl carbonate, dipentyl carbonate, methylethyl carbonate, methylpropyl carbonate and ethylpropyl carbonate,
wherein the dispersant is a hydrotreated light distillate,
wherein the lubricant is composed of at least one selected from the group consisting of a hydrotreated heavy paraffinic distillate, a hydrotreated light paraffinic distillate, a solvent-dewaxed heavy paraffinic distillate, a solvent-dewaxed light paraffin distillate, a hydrotreated and dewaxed heavy paraffinic distillate or a hydrotreated and dewaxed light paraffinic distillate,
wherein the non-ionic surfactant is composed of at least one selected from the group consiting of sorbitan esters of fatty acids, polyetheyleneglycol esters of fatty acids and polyethyleneglycol sorbitan esters of fatty acids,
wherein the overbased sulfonate-base detergent is composed of a compound of CAS Registration No. 68783-96-0 or a compound of CAS Registration No. 115733-10-3.

2. The fuel additive for a heavy fuel oil according to claim 1, wherein the non-ionic surfactant is composed of at least one selected from the group consisting of sorbitan monooleate, sorbitan monolaurate, or polyethyleneglycol sorbitan monooleate.

3. A fuel oil comprising a heavy fuel oil and the fuel additive for a heavy fuel oil according to any one of claims 1 to 2.

4. The fuel oil according to claim 3, wherein the content of the fuel additive for a heavy fuel oil in the fuel oil is 0.001 to 0.5 parts by weight per 100 parts by weight of the heavy fuel oil.

## Patentansprüche

1. Kraftstoffzusatz für ein schweres Heizöl in Form einer Zusammensetzung, wobei der Kraftstoffzusatz umfasst:
20 bis 25 Gew.-% einer öllöslichen Metallverbindung; 30 bis 35 Gew.-% eines Sauerstoffträgers; 15 bis 20 Gew.-% eines Dispergiermittels; 3 bis 7 Gew.-% eines Schmiermittels; 8 bis 15 Gew.-% eines nichtionischen Tensids; und 7 bis 15 Gew.-% eines überbasischen Detergens auf Sulfonatbasis, bezogen auf das Gesamtgewicht der Zusammensetzung,
wobei die öllösliche Metallverbindung ein Calciumalkylbenzolsulfonat ist und die Alkylgruppe 8 bis 50 Kohlenstoffatome aufweist,
wobei der Sauerstoffträger aus mindestens einer Verbindung zusammengesetzt ist, die aus der Gruppe ausgewählt ist, die aus Dimethylcarbonat, Diethylcarbonat, Dipropylcarbonat, Diiosopropylcarbonat, Dibutylcarbonat, Dipentylcarbonat, Methylethylcarbonat, Methylpropylcarbonat und Ethylpropylcarbonat besteht,
wobei das Dispergiermittel ein hydrobehandeltes Leichtdestillat ist,
wobei das Schmiermittel zusammengesetzt ist aus mindestens einem Mittel aus der Gruppe bestehend aus einem hydrobehandelten schweren paraffinischen Destillat, einem hydrobehandelten leichten paraffinischen Destillat, einem lösungsmittelentparaffinierten schweren paraffinischen Destillat, einem lösungsmittelentparaffinierten leichten paraffinischen Destillat, einem hydrobehandelten und entparaffinierten schweren paraffinischen Destillat oder einem hydrobehandelten und entparaffinierten leichten paraffinischen Destillat,
wobei das nichtionische Tensid aus mindestens einer Verbindung zusammengesetzt ist, die aus der Gruppe ausgewählt ist, die aus Sorbitanestern von Fettsäuren, Polyethylenglykolestern von Fettsäuren und Polyethylenglykolsorbitanestern von Fettsäuren besteht,
wobei das überbasische Detergens auf Sulfonatbasis aus einer Verbindung der CAS-Registrierungsnummer 68783-96-0 oder einer Verbindung der CAS-Registrierungsnummer 115733-10-3 zusammengesetzt ist.

2. Kraftstoffzusatz für ein schweres Heizöl nach Anspruch 1, wobei das nichtionische Tensid aus mindestens einem Stoff zusammengesetzt ist, der aus der Gruppe ausgewählt ist, die aus Sorbitanmonooleat, Sorbitanmonolaurat oder Polyethylenglykolsorbitanmonooleat besteht.

3. Heizöl, umfassend ein schweres Heizöl und den Kraftstoffzusatz für ein schweres Heizöl nach einem der Ansprüche 1 bis 2.

4. Heizöl nach Anspruch 3, wobei der Gehalt des Kraftstoffzusatzes für ein schweres Heizöl in dem Heizöl 0,001 bis 0,5 Gewichtsteile pro 100 Gewichtsteile des schweren Heizöls beträgt.

## Revendications

1. Additif de carburant pour un fioul lourd sous forme de composition, l'additif de carburant comprenant :
20 à 25% en poids d'un composé métallique soluble dans l'huile ; 30 à 35% en poids d'un véhicule oxygéné ; 15 à 20% en poids d'un dispersant ; 3 à 7% en poids d'un lubrifiant; 8 à 15% en poids d'un agent tensioactif non ionique ; et 7 à 15% en poids d'un détergent surbasique à base de sulfonate, par rapport au poids total de la composition,
le composé métallique soluble dans l'huile étant un alkylbenzènesulfonate de calcium et le groupe alkyle ayant 8 à 50 atomes de carbone,
le véhicule oxygéné étant composé d'au moins un élément choisi dans le groupe constitué par le carbonate de diméthyle, le carbonate de diéthyle, le carbonate de dipropyle, le carbonate de diiosopropyle, carbonate de dibutyle, carbonate de dipentyle, carbonate de méthyléthyle, carbonate de méthylpropyle et carbonate d'éthylpropyle,
le dispersant étant un distillat léger hydrotraité,
le lubrifiant étant composé d'au moins un élément choisi dans le groupe constitué par un distillat paraffinique lourd hydrotraité, un distillat paraffinique léger hydrotraité, un distillat paraffinique lourd déparaffiné au solvant, un distillat paraffinique léger déparaffiné au solvant, un distillat paraffinique lourd hydrotraité et déparaffiné ou un distillat paraffinique léger hydrotraité et déparaffiné,
l'agent tensioactif non ionique étant composé d'au moins un élément choisi dans le groupe constitué par les esters de sorbitane d'acides gras, les esters de polyéthylèneglycol d'acides gras et les esters de sorbitane de polyéthylèneglycol d'acides gras,
le détergent surbasique à base de sulfonate étant composé d'un composé du numéro d'enregistrement CAS. 68783-96-0 ou un composé du numéro d'enregistrement CAS 115733-10-3.

2. Additif de carburant pour un fioul lourd selon la revendication 1, l'agent tensioactif non ionique étant composé d'au moins un élément choisi dans le groupe constitué par le monooléate de sorbitane, le monolaurate de sorbitane ou le monooléate de sorbitane polyéthylèneglycol.

3. Fioul comprenant un fioul lourd et l'additif pour un fioul lourd selon l'une des revendications 1 à 2.

4. Fioul selon la revendication 3, dans lequel la teneur en additif pour un fioul lourd dans le fioul est de 0,001 à 0,5 partie en poids pour 100 parties en poids du fioul lourd.
